# EUROPEAN PATENT SPECIFICATION

(11) **EP 2 262 945 B1**
(45) Date of publication and mention of the grant of the patent: **13.03.2013**
(21) Application number: 09725488.2
(22) Date of filing: 27.03.2009
(51) Int. Cl.: D06P 1/38, D06P 1/382, D06P 1/384, D06P 3/00, D06P 3/24, D06P 3/66, D06P 1/16, D06P 1/18, D06P 1/19, D06P 1/20, D06P 1/41, D06P 1/42, D06P 1/44, D06P 3/26, D06P 3/48, D01F 1/04

(54) **INFLUENCING THE NEAR INFRARED REFLECTANCE OF DYED TEXTILE MATERIALS**
BEEINFLUSSUNG DER NAHINFRAROTREFLEXION GEFÄRBTER TEXTILSTOFFE
ACTION SUR LA RÉFLECTANCE DES MATÉRIAUX TEXTILES COLORÉS DANS L'INFRAROUGE PROCHE

(30) Priority: 28.03.2008 EP 08153509; 28.03.2008 EP 08153510; 28.03.2008 EP 08153511; 28.03.2008 EP 08153512; 28.03.2008 EP 08153513
(43) Date of publication of application: 22.12.2010
(73) Proprietor: Clariant Finance (BVI) Limited, Road Town, Tortola (VG)
(72) Inventor: NUSSER, Rainer, 79395 Neuenburg (DE); LEILER, Martin, Samutprakarn 10280 (TH); LOTTENBACH, Roland, CH-9422 Staad (CH); HUEBNER, Hans-Jürgen, CH-6645 Brione s. Minusio (CH)
(74) Representative: Hütter, Klaus
(86) International application number: PCT/EP2009/053696
(87) International publication number: WO 2009/118419

(56) References cited:
- EP-A- 0 200 131
- EP-A- 0 226 198
- EP-A- 0 273 300
- EP-A- 1 111 124
- WO-A-2005/017047
- WO-A-2005/113886
- WO-A-2007/090739
- DE-A1- 1 469 603
- DE-A1- 2 163 427
- DE-A1- 2 422 968
- DE-A1- 2 633 615
- DE-A1- 2 834 998
- DE-A1- 3 247 612
- DE-A1-102006 019 553
- DE-B1- 2 311 130
- DE-T2- 60 123 369
- US-A- 3 977 827
- US-A- 4 074 970
- US-A- 4 198 204
- DATABASE WPI Week 200650 Thomson Scientific, London, GB; AN 2006-484919 XP002493870 & JP 2006 176941 A (SEIREN CO LTD) 6 July 2006 (2006-07-06)

## Description

The invention concerns dyed textile materials having, compared with the same, undyed textile materials, an increased or at least equivalent reflectance of electromagnetic radiation in the near infrared (NIR), in particular dyed textile materials having increased or at least equivalent reflectance of electromagnetic radiation in the region of electromagnetic radiation of wavelength 700 nm to 1100 nm.

Surfaces coloured for aesthetic or else for technical reasons, in particular having a dark colour, and exposed to sunlight have the usually unpleasant property of heating up to a greater or lesser extent. Specifically in comparatively small enclosed spaces, as in a closed vehicle for example, the solar heating-up of surfaces is perceived as extremely unpleasant. The insolated areas heat up to a greater or lesser extent, depending on their degree of solar absorption, and emit their heat as thermal radiation into the interior. Outerwear is another arena where heating up due to insolation can become very unpleasantly noticeable.

DE 60123 369 T2 discloses a NIR reflecting composite piment. EP93377 and JP2006-348414 disclose a textile material coated with a polymer embedding metal particles which reflect thermal radiation. DE19540682 describes a thermally reflective coating comprising binder, pigments and solvent and/or water to control the heating up of materials coated therewith. WO02/12405 discloses a coated sheetlike article having reduced solar absorption wherein the coating consists of a pigment and a binder system. WO02/12405 is another instance where the binding system is mainly responsible for reflecting the NIR radiation. These processes all lead to coated textile materials which are extremely unpleasant when used as surfaces of seats and the like, but in particular when used as a textile material for apparel. The coatings often contain metal particles and/or inorganic pigments which largely contain metals.

It is therefore desirable to finish or dye textile materials such that they only heat up minimally, if at all, on irradiation, in particular on solar irradiation, or even reflect thermal radiation. But in the process the wearing comfort or the handle of these textile materials must not change.

It has now been found that dyeing or printing textile materials with ordinary dyes customary for the particular type of fibre while using the dyeing and/or printing processes customary for the particular type of fibre lead only to a minimal reduction, if at all, in NIR reflectance in the region of electromagnetic radiation of wavelength 700 nm to 1100 nm or even lead to an increased NIR reflectance in the region of electromagnetic radiation of wavelength 700 nm to 1100 nm compared with the undyed substrate on using metal-free dyes.

The present invention accordingly describes a process for minimally reducing, retaining or increasing the NIR reflectance, preferably increasing the NIR reflectance, in the region of electromagnetic radiation of wavelength 700 nm to 1100 nm of textile material in relation to the undyed and untreated textile material while using dyes for the type of fibre in question and while using the customary dyeing and/or printing processes for the type of fibre in question, characterized in that metal-free dyes are used, as hereinafter defined.

The invention also describes a dyeing process using dyes for the type of fibre in question and using the customary dyeing and/or printing processes for the type of fibre in question for minimally reducing, retaining or increasing the NIR reflectance, preferably increasing the NIR reflectance, in the region of electromagnetic radiation of wavelength 700 nm to 1100 nm of textile material in relation to the undyed and untreated textile material, characterized in that metal-free dyes are used, as hereinafter defined.

The invention also describes a textile material which is dyed by a dyeing process using dyes for the type of fibre in question and using the customary dyeing and/or printing processes for the type of fibre in question for minimally reducing, retaining or increasing the NIR reflectance, preferably increasing the NIR reflectance, in the region of electromagnetic radiation of wavelength 700 nm to 1100 nm of textile material in relation to the undyed and untreated textile material, characterized in that metal-free dyes are used, as herein after defined.

Minimal reduction means that the reflectance does not decrease by more than 5%age points (absolute) compared with the untreated substrate (textile material).

Increasing the NIR reflectance means that the reflectance of the NIR of the treated substrate (textile material) is higher, preferably by more than 2%age points (absolute), more preferably by more than 5%age points (absolute) compared with the untreated substrate (textile material).

The invention provides the use of dyes for the type of fibre in question for minimally reducing, retaining or increasing the NIR reflectance, preferably increasing the NIR reflectance, in the region of electromagnetic radiation of wavelength 700 nm to 1100 nm of textile material in relation to the undyed and untreated textile material, characterized in that customary dyeing and/or printing processes for the type of fibre in question are used and characterized in that the dyes are metal-free and are acid dyes having one of the following structures (A-I), (A-II), (A-III), (A-IV) or (A-V) where
- A: is an unsubstituted or substituted naphthyl radical or an unsubstituted or substituted phenyl radical,
- R³²: is hydrogen, hydroxyl, amino or an unsubstituted or substituted naphthyl radical or an unsubstituted or substituted phenyl radical, and
- n: is 1, 2 or 3,
where
- A: is an unsubstituted or substituted naphthyl radical or an unsubstituted or substituted phenyl radical,
- R³³: is hydrogen, hydroxyl, amino or an unsubstituted or substituted naphthyl radical or an unsubstituted or substituted phenyl radical, and
- n: is 1, 2 or 3,
where
- R³⁴, R³⁵, R³⁶, R³⁷: are each hydrogen, hydroxyl, amino, substituted or unsubstituted C₁ to C₄ alkyl, or an unsubstituted or substituted naphthyl radical or an unsubstituted or substituted phenyl radical and the dye of formula A-(III) bears one, two or three sulpho groups,
where
- A, R³⁸, R³⁹: are each hydrogen, hydroxyl, amino, substituted or unsubstituted C₁ to C₄ alkyl, or an unsubstituted or substituted naphthyl radical or an unsubstituted or substituted phenyl radical and the dye of formula A-(IV) bears one, two or three sulpho groups,
where
- R⁴⁰, R⁴¹, R⁴²: are each hydrogen, hydroxyl, amino, substituted or unsubstituted C₁ to C₄ alkyl, or an unsubstituted or substituted naphthyl radical or an unsubstituted or substituted phenyl radical,
- m: is 0, 1, 2 or 3 and the dye of formula (A-V) bears one, two or three sulpho groups,

or are basic dyes having one of the following structures (B-I), (B-II), (B-III), or (B-IV) where
- R⁴³ and R⁴⁴: are independently substituted or unsubstituted C₁ to C₄ alkyl, substituted or unsubstituted -(C₁₋₄ alkylene)-N⁺-(C₁₋₄ alkyl)₂, the dye of the formula (B-I) being at least singly or doubly positively charged;
where
- R⁵⁵ and R⁵⁶: are independently substituted or unsubstituted C₁ to C₄ alkyl, substituted or unsubstituted -N-(C₁₋₄ alkyl)₂;
where
- R⁵⁷ and R⁵⁸: are independently substituted or unsubstituted phenyl, substituted or unsubstituted naphthyl, and
- R⁵⁹: is independently substituted or unsubstituted phenyl, substituted or unsubstituted naphthyl or =N⁺H₂;
where
- R⁶⁰: is (C₁₋₄ alkyl)-C(O)NH₂
- R⁶¹: is C₁₋₄ alkyl or C₁₋₄ alkoxy, and
- R⁶²: is substituted or unsubstituted phenyl, substituted or unsubstituted naphthyl,

or are disperse dyes having the following formula (C-1) or (C-2) or (C-3) or (C-4) or (C-5) or (C-6) or (C-7) or (C-8) or (C-9) or (C-10) or (C-11) or
(C-12): where
- R₁: is hydrogen, halogen, nitro or cyano
- R₂: is hydrogen, halogen, nitro or cyano
- R₃: is hydrogen, halogen, C₁-C₄-alkoxy or C₁-C₄-alkyl
- R₄: is hydrogen, C₁-C₄-alkyl,
- R₅: is hydrogen, unsubstituted or hydroxyl-, cyano-, C₁-C₄-alkylcarbonyloxy-substituted C₁-C₄-alkyl or C₁-C₄-alkenyl,
- R₆: is unsubstituted or hydroxyl-, cyano-, C₁-C₄-alkylcarbonyloxy-, C₁-C₄-alkoxycarbonyl-substituted C₁-C₄-alkyl or C₁-C₄-alkenyl,
- R₇: is nitro, C₁-C₄-alkoxy or the radical -SO₂CH₃,
- R₈: is hydrogen or C₁-C₄-alkyl,
- R₉: is hydrogen or C₁-C₄-alkyl,
- R₁₀: is unsubstituted or hydroxyl- or cyano-substituted C₁-C₄-alkyl,
- R₁₁: is unsubstituted C₁-C₄-alkyl or C₁-C₄-alkyl substituted by the radical -O-COR₁₂, where R₁₂ is C₁-C₄-alkyl;
where
- R₁₃: is C₁-C₄-alkyl,
- R₁₄: is C₁-C₄-alkyl, and
Halogen represents the halogen atoms; where the rings A and B may be further substituted; where
- R₁₅: is C₁-C₄-alkyl and
the rings C and D may be further substituted; where
- R₁₆: is unsubstituted or hydroxyl- or cyano-substituted C₁-C₄-alkyl,
- R₁₇: is unsubstituted C₁-C₄-alkyl or C₁-C₄-alkyl substituted by the radical -O-COR₁₈, where R₁₈ is C₁-C₄-alkyl,
- R₃₂: is nitro, C₁-C₄-alkoxy or the radical -SO₂CH₃, and
- R₃₃: is hydrogen or C₁-C₄-alkyl;
where
- R₁₉: is C₁-C₄-alkyl,
- R₂₀: is C₁-C₄-alkyl,
- R₂₁: is C₁-C₄-alkyl, and
- R₂₂: is C₁-C₄-alkyl or the radical -NHCOR₂₃ where R₂₃ is C₁-C₄-alkyl;
where R₂₄ is halogen; where
- R₂₅: is cyano, nitro or halogen,
- R₂₆: is halogen,
- R₂₇: is unsubstituted or hydroxyl-substituted C₁-C₄-alkyl, and
- R₂₈: is unsubstituted or hydroxyl-substituted C₁-C₄-alkyl, and
the naphthyl ring E may be further substituted,
and/or where
- R₂₉: is C₁-C₄-alkyl or the radical NHCOR₁₇ where R₁₇ is C₁-C₄-alkyl,
- R₃₀: is C₁-C₄-alkyl or C₁-C₄-alkylcarbonyloxy-C₁-C₄-alkyl, and
- R₃₁: is C₁-C₄-alkyl or C₁-C₄-alkylcarbonyloxy-C₁-C₄-alkyl,

or are reactive dyes having one of the following structures (E-I), (E-II), (E-III), (E-IV), (E-V) or (E-VI) where
- A: is an unsubstituted or substituted naphthyl radical or an unsubstituted or substituted phenyl radical,
- R⁶³: is hydrogen, hydroxyl, amino, an amine substituted by unsubstituted or substituted naphthyl or by unsubstituted or substituted phenyl, or an unsubstituted or substituted naphthyl radical or an unsubstituted or substituted phenyl radical,
- n: is 1 or 2 and the dye of formula (E-I) bears one or two fibre-reactive groups;
where
- A: is an unsubstituted or substituted naphthyl radical or an unsubstituted or substituted phenyl radical,
- R⁶⁴: is hydrogen, hydroxyl, amino, an amine substituted by unsubstituted or substituted naphthyl or by unsubstituted or substituted phenyl, or an unsubstituted or substituted naphthyl radical or an unsubstituted or substituted phenyl radical,
- n: is 1, 2 or 3 and the dye of formula (E-II) bears one or two fibre-reactive groups;
where
- R⁶⁵, R⁶⁶, R⁶⁷, R⁶⁸: are each hydrogen, hydroxyl, amino, substituted or unsubstituted C₁ to C₄ alkyl, or an unsubstituted or substituted naphthyl radical or an unsubstituted or substituted phenyl radical and the dye of formula (E-III) bears one, two or three sulpho groups and also one or two fibre-reactive groups;
where
- A, R⁶⁹, R⁷⁰: are each hydrogen, hydroxyl, amino, an amine substituted by unsubstituted or substituted naphthyl or by unsubstituted or substituted phenyl, or an unsubstituted or substituted naphthyl radical or an unsubstituted or substituted phenyl radical and the dye of formula (E-IV) bears one, two or three sulpho groups and also one or two fibre-reactive groups;
where
- R⁷¹, R⁷², R⁷³: are each hydrogen, hydroxyl, amino, substituted or unsubstituted C₁ to C₄ alkyl, or an unsubstituted or substituted naphthyl radical or an unsubstituted or substituted phenyl radical
- m: is 0, 1, 2 or 3 and the dye of formula (E-V) bears one, two or three sulpho groups and also one or two fibre-reactive groups;
where
- A: in each occurrence is independently an unsubstituted or substituted naphthyl radical or an unsubstituted or substituted phenyl radical,
- R⁷⁴: is hydroxyl, amino, an amine substituted by unsubstituted or substituted naphthyl or by unsubstituted or substituted phenyl, or an unsubstituted or substituted naphthyl radical or an unsubstituted or substituted phenyl radical,
- n: is 1 or 2 and the dye of formula (E-VI) bears one or two fibre-reactive groups.

Preferably the textile material which is dyed with the metal-free acid dyes which have the structures (A-I), (A-II), (A-III), (A-IV) or (A-V) consists of nylon or wool, and synthetic PA6 (nylon-6) or else PA66 (nylon-6,6) can be used in the present invention. The substrate to be dyed can be for example in the form of sheetlike or threadlike structures, i.e. in the form of yarn, woven fabric, knitted fabric or carpet. Fully-fashioned dyeings are even very readily possible on delicate substrates, for example lambswool, cashmere, alpaca and mohair. The present invention is particularly useful for dyeing fine-denier fibres (microfibres).

Dyeing using the dyes which have the structures (A-I), (A-II), (A-III), (A-IV) or (A-V) is carried out in accordance with known processes; reference is made by way of example to the dyeing processes described in Ullmanns Encyklopädie der technischen Chemie, 4th edition, 1982, Volume 22, pages 658-673 or in the book by M. Peter and H.K. Rouette, Grundlagen der Textilveredlung, 13th edition, 1989, pages 535-556 and 566-574. Preference is given to dyeing by the exhaust method at a temperature of 30 to 140°C, more preferably 80 to 120°C and most preferably at a temperature of 80 to 100°C, and at a liquor ratio of 3:1 to 40:1. The dyes according to the invention can also be applied by printing, whether by traditional (classic) textile-printing processes or else by contactless printing, as by the ink jet process for example.

Useful anions for the dyes of the structures (B-I), (B-II), (B-III), or (B-IV) include chlorides, bromides, sulphates, carbonates and organic carboxylates. Dyes of the structures (B-I), (B-II), (B-III), or (B-IV) containing free basic groups can also be converted into water-soluble salts by converting the dyes which contain free basic groups with inorganic or organic acids. As examples there may be mentioned for example acetic acid, lactic acid, formic acid, hydrochloric acid, sulphuric acid.

Preferred textile material which is dyed by the dyes of the structures (B-I), (B-II), (B-III), or (B-IV) consists of polyacrylonitrile fibres, the so-called polyacrylic fibres or acrylic fibres. These preferred polyacrylonitrile fibres consist of not less than 85% of acrylonitrile units and are preferably terpolymers composed of acrylonitrile (89-95%), a nonionic comonomer (4-10%, for example vinyl chloride, methyl methacrylate) and an ionic comonomer (0.5-1%, for example vinylsulphonic acid, styrenesulphonic acid, vinylpyridine). Textile materials composed of anionically modified polyester fibres can also be used.

Dyeing using the dyes of the structures (B-I), (B-II), (B-III), or (B-IV) is carried out in accordance with known processes, described for example in M. Peter and H.K. Rouette: "Grundlagen der Textilveredelung; Handbuch der Technologie, Verfahren und Maschinen", 13th revised edition, 1989, Deutscher Fachverlag GmbH, Frankfurt/Main, Germany, ISBN 3-87150-277-4, wherein pages 602 to 606 (chapters 7.222.35, 7.222.351 and 7.222.351.1) are of particular interest. The exhaust process or else the padding process can be used.

The dyes of the structures (B-I), (B-II), (B-III) or (B-IV) according to the present invention can also be applied by printing, whether with conventional (classic) textile printing processes or else by contactless printing, as by ink jet printing for example.

The disperse dyes are dyes which are a sparing solubility in water, i.e. not more than 200 mg per litre, and which are used together with dispersants in a very finely ground state for dyeing and printing semisynthetic or synthetic hydrophobic fibre materials, preferably for dyeing and printing synthetic hydrophobic fibre materials. In the present invention, the molecularly dissolved portions of the dyes penetrate in the dyebath into the fibre by diffusion, form a solid solution therein and thereby produce fast dyeings.

The disperse dyes are particular disperse dyes selected from the azo, bisazo, nitro, anthraquinone, polymethine, coumarin, and naphthalimide series.

As to the foregoing disperse dyes of formulae (C-1) to (C-12):
C₁-C₄-Alkyl as such and as a radical in C₁-C₄-alkylcarbonylamino or C₁-C₄-alkylcarbonyloxy is methyl, ethyl, propyl, isopropyl, n-butyl, isobutyl, sec-butyl or tert-butyl.

C₁-C₄-Alkoxy as such or as a radical in C₁-C₄-alkoxycarbonyl is for example methoxy, ethoxy, propoxy or butoxy.

Halogens R₁, R₃, R₂₅ and R₂₆ are for example bromine or preferably chlorine.

Halogens R₂ and R₂₄ are for example chlorine or preferably bromine.

Halogen in the formula (C-3) is for example bromine or preferably chlorine.

C₁-C₄-Alkyls R₅, R₆ and R₁₆ are propyl or isopropyl and in particular ethyl.

C₁-C₄-Alkyls R₁₃, R₁₅, R₁₈, R₂₂, R₂₃, R₈, R₃₁ and R₃₃ are preferably ethyl and especially methyl.

C₁-C₄-Alkyls R₁₄, R₁₉, R₂₁, R₁₁, R₃₀ and R₂₅ are preferably methyl and especially ethyl.

C₁-C₄-Alkyls R₁₉, R₂₀, R₂₇ and R₂₈ are preferably ethyl and especially propyl.

R₃₀ and R₃₁ are preferably C₁-C₄-alkyl.

R₂₆ is preferably nitro or the radical -SO₂CH₃.

The C₁-C₄-alkyl radicals are generally substituted one or two times with the aforementioned substituents.

The rings A to E may be independently substituted for example by C₁-C₄-alkyl, C₁-C₄-alkoxy, halogen, nitro, cyano or acylamino.

Preferably the textile material dyed with metal-free disperse dyes with the structures of the formula (C-1) or (C-2) or (C-3) or (C-4) or (C-5) or (C-6) or (C-7) or (C-8) or (C-9) or (C-10) or (C-11) or (C-12) consists of semisynthetic and preferably synthetic hydrophobic fibre materials.

Useful semisynthetic textile materials are in main secondary cellulose acetate, cellulose triacetate, polyamides and macromolecular polyesters and also blends thereof with cellulose.

Synthetic hydrophobic textile materials consist in the main of linear aromatic polyesters, for example those formed from terephthalic acid and glycols, in particular ethylene glycol, or condensate of terephthalic acid and 1,4-bis(hydroxymethyl)-cyclohexane, of polycarbonates, for example those of α,α-dimethyl-4,4'-dihydroxydiphenylmethane and phosgene, and of fibres based on polyvinyl chloride and polyamide.

The textile materials can be present as sheet or thread structures and can have been processed for example into yarns or woven, knitted or loop material. The textile materials can be present in the form of microfibres.

The dyeing or printing textile materials with metal-free disperse dyes with the structures of the formula (C-1) or (C-2) or (C-3) or (C-4) or (C-5) or (C-6) or (C-7) or (C-8) or (C-9) or (C-10) or (C-11) or (C-12) can be made by conventional processes, for example those in accordance with French patent application No. 1.445.371.

Typically, polyester fibre materials are dyed from an aqueous dispersion by the exhaust process in the presence of customary anionic or nonionic dispersants and in the presence or absence of customary swelling agents (carriers) in the temperature range from 65°C. to 140°C.

Secondary cellulose acetate is preferably dyed at a temperature from 65°C to 85°C and cellulose triacetate at temperatures up to 115°C.

The metal-free disperse dyes with the structures of the formula (C-1) or (C-2) or (C-3) or (C-4) or (C-5) or (C-6) or (C-7) or (C-8) or (C-9) or (C-10) or (C-11) or (C-12) are suitable for dyeing by the thermosol process, for the exhaust process, the continuous process and for printing as for modem imaging processes, for example thermal transfer printing, inkjet printing, hot melt inkjet printing or by conventional printing processes.

The thermosol process, the exhaust process and the continuous process are well-known dyeing processes and are described for example in M. Peter and H.K. Rouette: "Grundlagen der Textilveredelung; Handbuch der Technologie, Verfahren und Maschinen", 13th revised edition, 1989, Deutscher Fachverlag GmbH, Frankfurt/Main, Germany, ISBN 3-87150-277-4, wherein the following pages are of particular interest: pages 460-461, 482-495, 556-566 and 574-587.

The dyeings with metal-free disperse dyes with the structures of the formula (C-1) or (C-2) or (C-3) or (C-4) or (C-5) or (C-6) or (C-7) or (C-8) or (C-9) or (C-10) or (C-11) or (C-12) are carried out from an aqueous liquor by the exhaust process, and the liquor ratio can be chosen within wide limits, for example in the range from 4:1 to 100:1 and preferably in the range from 6:1 to 50:1.

The dyeing time is in the range from 20 to 90 minutes and preferably in the range from 30 to 60 minutes.

The dyeing liquors may additionally comprise further additives, for example dyeing auxiliaries, dispersants, wetting agents and antifoams.

The liquor may also comprise mineral acids, such as sulphuric acid or phosphoric acid, or advantageously also organic acids, for example formic acid or acetic acid and/or salts thereof, such as ammonium acetate, ammonium sulphate or sodium sulphate. The acids mainly serve to adjust the dyeing liquors to a pH which is preferably in the range from 4 to 5.

The metal-free disperse dyes with the structures of the formula (C-1) or (C-2) or (C-3) or (C-4) or (C-5) or (C-6) or (C-7) or (C-8) or (C-9) or (C-10) or (C-11) or (C-12) are usually present in the dyeing liquors in the form of a fine dispersion. Suitable dispersants for preparing this dispersion are for example anionic dispersants, such as aromatic sulphonic acid-formaldehyde condensates, sulphonated cresol oil-formaldehyde condensates, ligninsulphonates or copolymers of acrylic acid derivatives, preferably aromatic sulphonic acid-formaldehyde condensates or ligninsulphonate, or nonionic dispersants based on polyalkylene oxides, for example obtainable by polyaddition of ethylene oxide or propylene oxide. Suitable dispersants are further recited in US 4,895,981 or in US 5,910,624.

The dyes use metal-free dyes which contain as well as a colour-conferring component (chromophore) and contain a specific reactive component via which they react with functional groups on the fibre (for example hydroxyl groups in the case of cellulose or amide groups in the case of wool and nylons) and become covalently bonded thereto.

Reactive dyes come from the azo (monoazo, disazo), anthraquinone and phenoxazine series, and particularly preferred reactive dyes from the monoazo, disazo and anthraquinone series. The reactive component of the dyes which are used in the present invention comprises halogenated, unsaturated, usually heterocyclic radicals such as for example 1,3,5-triazines, pyrazines, pyrimidines, the halogen atoms reacting in an alkaline medium with hydroxyl groups on the cellulose by hydrogen halide elimination and formation of ester-type bonds, on the one hand and, on the other, hydrogensulphate or sulphamate esters, for example of 3-hydroxypropionamido and 2-hydroxyethylsulphonyl groups, these esters in an alkaline medium spontaneously detaching sulphate and converting into acrylamido or vinylsulphonyl groups which in turn combine with hydroxyl groups on the cellulose to form stable ethers.

Preferred substrates for use in the present invention are textile materials dyed with reactive dyes having one of the structures (E-I), (E-II), (E-III), (E-IV), (E-V) or (E-VI), and the substrates consisting of or containing natural or synthetic polyamides or natural or rejuvenated cellulose, such as cotton, filament viscose or staple viscose,

the most preferred substrate is textile material consisting of or containing cotton.

The dyes of the present invention can be used in dyeing liquors or in printing pastes according to any dyeing or printing method customary for reactive dyes. Preference is given to dyeing by the exhaust method, in which case a temperature interval of 30-98°C is used, but the temperature does depend on the identity of the reactive hook.

Hot-dyeing dyes (60-98°C) are not very reactive and have to be activated by high temperature and also strong alkali. They include for example monochlorotriazinyl, trichloropyrimidyl and tetrachloropyrimidyl dyes.

Cold-dyeing dyes (40-60°C) are highly reactive dyes having dichlorotriazinyl, chlorodifluoropyrimidyl, difluoropyrimidyl or dichloroquinoxaline hooks, which react with the fibre without strong alkali and at relatively low temperatures.

In accordance with a further aspect of the present invention there is a hydroxyl-containing or nitrogenous organic substrate dyed or printed in accordance with the dyeing or printing process with reactive dyes described above.

Also, there are substrates, in particular cellulose, nylons and animal fibres, preferably cotton, dyed or printed with such compounds.

Similarly paper and optionally pretreated substrates containing cellulose, nylons or animal fibres and printed with ink jet printing inks containing such compounds, their salts or mixtures.

Conventional (classic) printing processes are known per se and differ in the way the printing ink or paste is transferred to the substrate. For example, inks or pastes can be applied by raised type as for example in letterpress and flexographic printing, from a planar surface in lithographic printing, from a recessed surface (intaglio) or through a stencil (silk screen). Different methods of application and different substrates require different properties of the ink.

In the inkjet printing process, individual droplets of the ink are sprayed from a nozzle onto a substrate in a controlled manner. The continuous inkjet method and the drop-on-demand method are employed predominantly for this purpose. In the case of the continuous inkjet method, the droplets are produced continuously and droplets not needed for printing are diverted into a collecting vessel and recycled. In the case of the discontinuous drop-on-demand method, by contrast, droplets are generated and printed as desired, i.e. droplets are only generated when this is necessary for printing. The droplets may be generated for example by means of a piezo inkjet head or by means of thermal energy (bubble jet).

In hot melt inkjet printing, solid hot melt inks are loaded into a printer capable of melting the ink in the inkjet printer head, injecting the liquid ink which quickly resolidifies upon impacting a substrate. Conventional hot melt inkjet printers operate with a printing head and inkjet temperature of about 120 to 150°C. At these temperatures, the solid ink melts to form a liquid of low viscosity, generally 8 to 25 cP at the jetting temperature.

In the inkjet printing process, individual droplets of the ink are sprayed from a nozzle onto a substrate in a controlled manner. The continuous inkjet method and the drop-on-demand method are employed predominantly for this purpose. In the case of the continuous inkjet method, the droplets are produced continuously and droplets not needed for printing are diverted into a collecting vessel and recycled. In the case of the discontinuous drop-on-demand method, by contrast, droplets are generated and printed as desired, i.e. droplets are only generated when this is necessary for printing. The droplets may be generated for example by means of a piezo inkjet head or by means of thermal energy (bubble jet).

In hot melt inkjet printing, solid hot melt inks are loaded into a printer capable of melting the ink in the inkjet printer head, injecting the liquid ink which quickly resolidifies upon impacting a substrate. Conventional hot melt inkjet printers operate with a printing head and inkjet temperature of about 120 to 150°C. At these temperatures, the solid ink melts to form a liquid of low viscosity, generally 8 to 25 cP at the jetting temperature.

The present invention additionally provides a method of increasing the sun protection factor (SPF) rating of cellulosic or protein fiber or fabric.

Cellulosic fibres may be any fibres of plant origin such as cotton, viscose, flax, linen, rayon or the like or composites thereof. Also, composites can be with polyester, polyamides, polyacrylonitriles or the like. Also, composites can be with polyester, polyamide or the like.

Protein fibres may be any fibres of animal origin such as wool, mohair, silk, cashmere, angora or the like or composites thereof. Also, composites can be with polyester, polyamide or the like.

The fabrics may be made of any fibres of plant origin such as cotton, viscose, flax, linen, rayon or the like or composites thereof. Also, composites can be with polyester, polyamides, polyacrylonitriles or the like.

The fabrics may be made of any fibres of animal origin such as wool, mohair, silk, cashmere, angora or the like or composites thereof. Also, composites can be with polyester, polyamide or the like.

Essentially, the SPF protection of a fabric depends on the "Cover Factor" of the fabric. The Cover Factor may be defined as the percentage of the fabric surface that is covered by the yarns of the fabric. If one assumes that the yarns employed to weave or knit the fabric are completely opaque to UVR radiation (which is not the case in reality) then the fabric SPF would be simply related to Cover Factor by the following formula: $Fabric SPF = \frac{100}{100 - Cover Factor}$

The method of increasing the SPF rating of fibers or fabrics comprises the use of the compounds (I) to (IV) as described in WO94/04515. WO94/04515.

The method of increasing the SPF rating of fibers or fabrics comprises applying to the fibers or fabrics one or more compounds of formula wherein A signifies -NH- or -SO₂- and if A signifies -NH- then B signifies on of the following moieties and if B singifies -SO₂- then B signifies on of the following moieties

-CH=CH-OSO₃H

-CH₂ - CH₂ - OSO₃H

-NH-CH₂-CH₂-OSO₃H

wherein R independently is selected from -OH, -NH₂, -SO₃⁻M⁺, -SO₃H, alkyl, alkoxy, alkanoyl, alkylcarboxylate, -S-alkyl, -CF₃, -N-di-alkyl;
n = 0, 1, 2, 3 or 4,
M⁺ = cation,
X = H or CI, F, Br and is independently selected,
Y=XorR.

Preferably the method of increasing the SPF rating of fibers or fabrics comprises applying to the fibers or fabrics one or more compounds of formula wherein B is selected from one of the following moieties (i) or (ii): wherein R independently is selected from -OH, -NH₂, -SO₃⁻M⁺, -SO₃H, alkyl, alkoxy, alkanoyl, alkylcarboxylate, -S-alkyl, -CF₃, -N-di-alkyl;
n = 0, 1, 2, 3 or 4,
M⁺ = cation,
X = H or CI, F, Br and is independently selected,
Y=XorR.

The method of increasing the SPF rating of fibers or fabrics comprises applying to the fibers or fabrics one or more of said compounds an application of less than 3% of a said compound on weight of fiber or fabric produces an SPF rating of greater than 20.

The SPF increasing compounds may be applied to cotton by either exhaustion or pad methods, or by the same methods which are usual for the respective fiber or fabric respectively. SPF increasing compounds may be applied may be applied before, during are after the dyeing. SPF increasing compounds are preferably applied during the dyeing operation.

### Compounds of formulae

wherein the substituents have the meaning as described above are useful as UVR absorber compounds and can be applied to fabrics of any weight. Typically, they are suitable for application to light weight summer fabrics and to heavier fabric up to and including industrial weight fabrics.

The process for increasing the SPF of the fibers and fabrics comprises the use and the application of the compounds (I) to (IV) as described in WO94/04515.

These compounds as described in WO94/04515 especially the compounds of the formula (I) to (IV) as described in WO94/04515 and the method and process for increasing the SPF of the fibers and fabrics is described in e.g. WO94/04515.

In the description and in the following examples and claims, parts and % are by weight, unless otherwise stated. The examples which follow illustrate the invention.

### EXAMPLE A-1 AND USE EXAMPLE A-A

A dyebath at 40°C, consisting of 2000 parts of water, 1 part of a weakly cation-active levelling agent which is based on an ethoxylated aminopropyl fatty acid amide and which has affinity for dye, 2.2 parts of the dye of C.I. Acid Yellow 218, and adjusted to pH 5 with 1-2 parts of 40% acetic acid is entered with 100 parts of nylon-6,6 fabric. After 10 minutes at 40°C, the dyebath is heated to 98°C at a rate of 1°C per minute and then left at the boil for 45-60 minutes. Thereafter it is cooled down to 70°C over 15 minutes. The dyeing is removed from the bath, rinsed with hot and then with cold water and dried.

The reflectance of the dyed substrate compared with the undyed substrate in the near infrared region is:

| **Substrate** | **Dye** | **Concentration** | **Reflectance at 800 nm** | **950 nm** | **1100 nm** |
|---|---|---|---|---|---|
| Nylsuisse nylon-6,6 | --- | --- | 89% | 88% | 87% |
| wool gabardine | ---- | --- | 85% | 85% | 84% |
| wool gabardine | C.I. Acid Yellow 218 | 2.2% | 89% | 88% | 87% |

Substrates dyed or printed with C.I. Acid Yellow 218 similarly to Use Examples B-G give the same measured results.

### USE EXAMPLE A-B

A dyebath at 40°C, consisting of 2000 parts of water, 1 part of a weakly cation-active levelling agent which is based on an ethoxylated aminopropyl fatty acid amide and which has affinity for dye, 0.3 part of the dye of Use Example A and adjusted to pH 5.5 with 1-2 parts of 40% acetic acid is entered with 100 parts of nylon-6,6 fabric. After 10 minutes at 40°C, the dyebath is heated to 120°C at a rate of 1.5°C per minute and then left at this temperature for 15-25 minutes. Thereafter it is cooled down to 70°C over 25 minutes. The dyeing is removed from the dyebath, rinsed with hot and then with cold water and dried. The result obtained is a yellow polyamide dyeing with good levelness and having good light and wet fastnesses.

### USE EXAMPLE A-C

A dyebath at 40°C, consisting of 4000 parts of water, 1 part of a weakly amphoteric levelling agent which is based on a sulphated, ethoxylated fatty acid amide and which has affinity for dye, 0.4 part of the abovementioned dye and adjusted to pH 5 with 1-2 parts of 40% acetic acid is entered with 100 parts of wool fabric. After 10 minutes at 40°C, the dyebath is heated to boiling at a rate of 1°C per minute and then left at the boil for 40-60 minutes. Thereafter it is cooled down to 70°C over 20 minutes. The dyeing is removed from the bath, rinsed with hot and then with cold water and dried.

### USE EXAMPLE A-D

100 parts of a woven nylon-6 material are padded with a 50°C liquor consisting of

| | |
|---|---|
| 40 | parts of the abovementioned dye, |
| 100 | parts of urea, |
| 20 | parts of a nonionic solubilizer based on butyldiglycol, |
| 15-20 | parts of acetic acid (to adjust the pH to 4), |
| 10 | parts of a weakly cation-active levelling agent which is based on an ethoxylated aminopropyl fatty acid amide and has affinity for dye, and |
| 810-815 | parts of water (to make up to 1000 parts of padding liquor). |

The material thus impregnated is rolled up and left to dwell in a steaming chamber under saturated steam conditions at 85-98°C for 3-6 hours for fixation. The dyeing is then rinsed with hot and cold water and dried. The result obtained is a blue nylon dyeing having good levelness in the piece and good light and wet fastnesses.

### USE EXAMPLE A-E

A textile cut pile sheet material composed of nylon-6 and having a synthetic base fabric is padded with a liquor containing per 1000 parts

| | |
|---|---|
| 1 | part of the abovementioned dye |
| 4 | parts of a commercially available thickener based on carob flour ether |
| 2 | parts of a nonionic ethylene oxide adduct of a higher alkylphenol |
| 1 | part of 60% acetic acid. |

This is followed by printing with a paste which per 1000 parts contains the following components:

| | |
|---|---|
| 20 | parts of commercially available alkoxylated fatty alkylamine (displace product) |
| 20 | parts of a commercially available thickener based on carob flour ether. |

The print is fixed for 6 minutes in saturated steam at 100°C, rinsed and dried.

### USE EXAMPLE A-F

3 parts of the abovementioned dye are dissolved in 82 parts of demineralized water and 15 parts of diethylene glycol at 60°C. Cooling down to room temperature gives an orange printing ink which is very highly suitable for ink jet printing on paper or polyamide and wool textiles.

### USE EXAMPLE A-G

A dyebath consisting of 1000 parts of water, 80 parts of calcined Glauber salt, 1 part of sodium nitrobenzene-3-sulphonate and 1 part of the abovementioned dye is heated to 80°C in the course of 10 minutes. Then, 100 parts of mercerized cotton are added. This is followed by dyeing at 80°C for 5 minutes and then heating to 95°C in the course of 15 minutes. After 10 minutes at 95°C, 3 parts of sodium carbonate are added, followed by a further 7 parts of sodium carbonate after 20 minutes and another 10 parts of sodium carbonate after 30 minutes at 95°C. Dyeing is subsequently continued at 95°C for 60 minutes. The dyed material is then removed from the dyebath and rinsed in running demineralized water for 3 minutes. This is followed by two washes for 10 minutes in 5000 parts of boiling demineralized water at a time and subsequent rinsing in running demineralized water at 60°C for 3 minutes and with cold tap water for one minute.

### EXAMPLES A-2 - A-34

Table 1 below contains dyes which were dyed or printed analogously to the use examples described under Example A-1 using the appropriate dyeing auxiliaries, and also the reflectance values of the respective dyed or printed substrates in the near infrared region:

**TABLE 1**

| **Example** | **Substrate** | **Dye** | **Concentration** | **Reflectance at 800 nm** | **950 nm** | **1100 nm** |
|---|---|---|---|---|---|---|
| **A-2** | nylon-6,6 | C.I. Acid Red 111 | 2.5% | 89% | 88% | 87% |
| **A-3** | nylon-6,6 | C.I. Acid Red 143 | 1.5% | 88% | 88% | 87% |
| **A-4** | nylon-6,6 | C.I. Acid Violet 48 | 2.2% | 75% | 87% | 86% |
| **A-5** | nylon-6,6 | C.I. Acid Blue 80 | 1.5% | 89% | 88% | 87% |
| **A-6** | nylon-6,6 | C.I. Acid Violet 54 | 2.2% | 89% | 88% | 87% |
| **A-7** | nylon-6,6 | C.I. Acid Yellow 256 | 1.5% | 89% | 88% | 87% |
| **A-8** | nylon-6,6 | C.I. Acid Yellow 199 | 1.5% | 80% | 85% | 87% |
| **A-9** | nylon-6,6 | C.I. Acid Yellow 49 | 1.5% | 89% | 88% | 87% |
| **A-10** | nylon-6,6 | C.I. Acid Brown 248 | 2.2% | 87% | 88% | 87% |
| **A-11** | nylon-6,6 | C.I. Acid Red 57 | 1.1% | 88% | 89% | 87% |
| **A-12** | nylon-6,6 | C.I. Acid Violet 126 | 2.0% | 89% | 88% | 87% |
| **A-13** | nylon-6,6 | C.I. Acid Blue 324 | 1.1% | 80% | 88% | 87% |
| **A-14** | nylon-6,6 | C.I. Acid Blue 45 | 1.5% | 89% | 88% | 87% |
| **A-15** | nylon-6,6 | C.I. Acid Yellow 42 | 1.5% | 89% | 88% | 87% |
| **A-16** | nylon-6,6 | C.I. Acid Red 260 | 3.0% | 89% | 89% | 87% |
| **A-17** | nylon-6,6 | C.I. Acid Red 415 | 3.0% | 89% | 88% | 87% |
| **A-18** | nylon-6,6 | C.I. Acid Orange 116 | 2.5% | 87% | 88% | 87% |
| **A-19** | nylon-6,6 | C.I. Acid Blue 280 | 3.0% | 80% | 84% | 86% |
| **A-20** | nylon-6,6 | C.I. Acid Green 25 | 2.0% | 85% | 88% | 87% |
| **A-21** | nylon-6,6 | C.I. Acid Yellow 236 | 2.5% | 89% | 88% | 87% |
| **A-22** | wool gabardine | C.I. Acid Yellow 236 | 2.0% | 81% | 81% | 81% |
| **A-23** | nylon-6,6 | Nylosan Rot S-3B | 2.0% | 86% | 87% | 87% |
| **A-24** | wool gabardine | Nylosan Rot S-3B | 4.0% | 81% | 85% | 84% |
| **A-25** | nylon-6,6 | Nylosan Navy S-3G | 0.5% | 77% | 81% | 85% |
| **A-26** | wool gabardine | Nylosan Navy S-3G | 0.5% | 80% | 83% | 84% |
| **A-27** | nylon-6,6 | C.I. Acid Yellow 17 | 1.5% | 89% | 88% | 87% |
| **A-28** | nylon-6,6 | C.I. Acid Yellow 172 | 3.0% | 89% | 88% | 87% |
| **A-29** | nylon-6,6 | C.I. Acid Red 37 | 1.0% | 88% | 88% | 87% |
| **A-30** | nylon-6,6 | C.I. Acid Yellow 19 | 2.2% | 87% | 88% | 87% |
| **A-31** | nylon-6,6 | C.I. Acid Blue 182 | 1.1% | 86% | 88% | 87% |
| **A-32** | nylon-6,6 | C.I. Acid Red 145 | 2.0% | 89% | 88% | 87% |
| **A-33** | nylon-6,6 | C.I. Acid Red 249 | 2.0% | 89% | 88% | 87% |
| **A-34** | nylon-6,6 | C.I. Acid Blue 129 | 2.0% | 85% | 88% | 87% |

### EXAMPLE B-1 (DYED IN ACCORDANCE WITH USE EXAMPLE B-A)

0.55 part of C.I. Basic Blue 22 is dissolved in 250 parts of demineralized water. 0.5 part of Ekalin F and 0.2 part of sodium acetate are added and the pH is adjusted to 4.5 with acetic acid. The dyebath is heated to 65°C and entered with 10 parts of Orlon 75. The dyebath is then heated to 80°C at a rate of 1°C/min and then to 105°C at 0.5-1°C/min. Dyeing is continued at 105°C for 60 min. The dyed fabric is then rinsed for 3 minutes with running cold water and subsequently for 3 minutes with running hot water and thereafter centrifuged and dried in a drying cabinet at 60°C.

The reflectance of the dyed substrate compared with the undyed substrate in the near infrared region is:

| **Substrate** | **Dye** | **Concentration** | **Reflectance at 800 nm** | **950 nm** | **1100 nm** |
|---|---|---|---|---|---|
| Orlon 75 | --- | --- | 90% | 90% | 90% |
| ditto | C.I. Basic Blue 22 | 1.1% | 86% | 89% | 89% |

### EXAMPLES B-2 - B-35

Table 2 below contains dyes which were dyed on Orlon 75 analogously to the Use Example B-A described under Example B-1 using the appropriate dyeing auxiliaries, and also the reflectance values of the respective dyed or printed substrates in the near infrared region:

**TABLE 2**

| **Example** | **Dye** | **Concentration** | **Reflectance at 800 nm** | **950 nm** | **1100 nm** |
|---|---|---|---|---|---|
| **B-2** | C.I. Basic Blue 1 | 1.5% | 86% | 88% | 89% |
| **B-3** | C.I. Basic Blue 3 | 1.0% | 85% | 85% | 86% |
| **B-4** | C.I. Basic Blue 26 | 2.2% | 88% | 89% | 89% |
| **B-5** | C.I. Basic Blue 67 | 0.8% | 86% | 86% | 85% |
| **B-6** | C.I. Basic Blue 11 | 0.8% | 87% | 85% | 84% |
| **B-7** | C.I. Basic Yellow 1 | 1.0% | 86% | 86% | 86% |
| **B-8** | C.I. Basic Yellow 2 | 1.5% | 86% | 86% | 86% |
| **B-9** | C.I. Basic Yellow 13 | 1.0% | 88% | 86% | 86% |
| **B-10** | C.I. Basic Yellow 106 | 0.8% | 85% | 85% | 86% |
| **B-11** | C.I. Basic Yellow 90 | 1.1% | 86% | 86% | 86% |
| **B-12** | C.I. Basic Orange 2 | 1.5% | 90% | 90% | 90% |
| **B-13** | C.I. Basic Orange 30 | 1.1% | 86% | 86% | 86% |
| **B-14** | C.I. Basic Red 1:1 | 1.5% | 88% | 86% | 86% |
| **B-15** | C.I. Basic Red 13 | 0.8% | 85% | 85% | 86% |
| **B-16** | C.I. Basic Red 18 | 1.5% | 85% | 85% | 86% |
| **B-17** | C.I. Basic Red 46 | 1.1% | 85% | 85% | 86% |
| **B-18** | C.I. Basic Green 1 | 1.0% | 84% | 85% | 86% |
| **B-19** | C.I. Basic Green 4 | 1.0% | 88% | 86% | 86% |
| **B-20** | C.I. Basic Brown 1 | 0.8% | 85% | 85% | 86% |

### EXAMPLE C-1 AND USE EXAMPLE C-A

17.5 parts of the dye C.I. Disperse Yellow 42 in the form of the moist presscake are wet ground by a known method with 32.5 parts of a commercially available dispersant based on ligninsulphonates and pulverized to a powder. 1.2 parts of this dyeing preparation are added to 2000 parts of demineralized water at 70°C, which contain 40 parts of ammonium sulphate. The pH of the dyebath is set to 5 with 85% formic acid. This dyebath is entered with 100 parts of cleaned woven polyester fibre fabric, the apparatus is sealed, and the temperature is raised to 130°C in the course of 20 min and dyeing is continued at 130°C for a further 40 min. After cooling, the woven polyester fibre fabric is removed from the dyebath, rinsed, soaped and reduction cleared in a conventional manner with sodium hydrosulphite. After thermofixing (180°C, 30 sec), a brilliant yellow dyeing is obtained with very good all-round fastness, especially fastness to light and sublimation, especially excellent wet fastness.

### USE EXAMPLE C-B

2.5 parts of the abovementioned dye are dissolved in a mixture of 20 parts of diethylene glycol and 77.5 parts of water at 25°C with stirring to obtain a printing ink suitable for inkjet printing.

### USE EXAMPLE C-C

A printing paste according to the invention consists of

| | |
|---|---|
| 500 g | of a thickener (bean gum ether, for example Indalca^{®}), |
| 10 g | of a fixation accelerant (e.g. Printogen^{®} HDN liq.), |
| 10 g | of a levelling agent (e.g. Lyogen^{®} CN liq.), |
| 10 g | of a buffering and dispersant system for dyeing (e.g. Opticid^{®} PB; 1:2) and also |
| 10 g | of C.I. Disperse Yellow 42 |

and water ad 1000 g.

(Indalca was purchased from Cesalpinia S.p.A., Italy; Lyogenn, Printogen and Opticid are trademarks of Clariant AG, Muttenz, Switzerland).

This printing paste is used for printing papery substrates, textile fibre materials and plastic films and plastic transparencies.

### USE EXAMPLE C-D

A polyester interlock fabric was printed with a conventional printing machine using the printing paste of **USE EXAMPLE C-C.** The printed fabric obtained is dried at 110°C for 3 minutes and then treated with hot steam at 175°C for 7 minutes. The fabric is rinsed with cold tap water for 5 minutes and then with demineralized water for 5 minutes. The fabric thus treated was reduction cleared in a bath containing 4 g/l of Na₂CO₃, 2 g/l of hydrosulphite sodium salt (85%) and 1 g/l of Lyogen^{®} DFT (trade mark of Clariant AG, Muttenz, Switzerland). Further rinsing for 15 minutes with tap water was followed by a final drying step. This leaves a polyester fabric having a brilliant red print with very good all-round fastness, especially fastness to light and sublimation, in particular excellent wetfastness.

### USE EXAMPLE C-E

The inkjet printing composition is preferably prepared by heating the medium to 40°C and then adding the abovementioned dye. The mixture is stirred until the dyes are dissolved. The composition is then cooled down to room temperature and the further ingredients are added.

The fractions of the individual components of the ink compositions
- 6 parts: of C.I. Disperse Yellow 42,
- 20 parts: of glycerol and
- 74 parts: of water.

This ink composition is used for printing papery substrates, textile fibre materials and plastic films and plastic transparencies.

### USE EXAMPLE C-F

A polyester interlock fabric was inkjet printed using the printing ink of **USE EXAMPLE C-E.** The printed fabric was treated analogously to the post printing treatment of **USE EXAMPLE C-D.** This gives a polyester fabric with a brilliant red print with very good all-round fastness, especially fastness to light and sublimation, in particular excellent wetfastness.

The reflectance of the dyed substrate compared with the undyed substrate in the near infrared region is:

| **Substrate** | **Dye** | **Concentration** | **Reflectance at 800 nm** | **950 nm** | **1100 nm** |
|---|---|---|---|---|---|
| Polyester, Tersuisse 9046 | --- | --- | 85% | 83% | 82% |
| Polyester, Tersuisse 9046 | C.I. Disperse Yellow 42 | 1.5% | 89% | 89% | 87% |

### EXAMPLES C-2 - C-35

Table 3 below contains dyes which were dyed or printed on polyester analogously to the use examples C-A to C-F described under Example C-1 using the appropriate dyeing auxiliaries, and also the reflectance values of the respective dyed or printed substrates in the near infrared region:

**TABLE3**

| **Example** | **Dye** | **Concentration** | **Reflectance at 800 nm** | **950 nm** | **1100 nm** |
|---|---|---|---|---|---|
| **C-2** | C.I. Disperse Orange 30 | 2.5% | 86% | 86% | 86% |
| **C-3** | C.I. Disperse Red 73 | 2.0% | 86% | 86% | 86% |
| **C-4** | C.I. Disperse Red 60 | 0.5% | 91% | 90% | 90% |
| **C-5** | C.I. Disperse Blue 56 | 0.8% | 86% | 86% | 85% |
| **C-6** | C.I. Disperse Blue 73 | 0.8% | 87% | 85% | 84% |
| **C-7** | C.I. Disperse Yellow 64 | 1.0% | 86% | 86% | 86% |
| **C-8** | C.I. Disperse Blue 354 | 1.0% | 85% | 86% | 85% |
| **C-9** | C.I. Disperse Red 86 | 1.1% | 93% | 89% | 89% |
| **C-10** | C.I. Disperse Violet 27 | 1.1% | 89% | 89% | 89% |
| **C-11** | C.I. Disperse Red 167:1 | 2.5% | 86% | 86% | 86% |
| **C-12** | C.I. Disperse Blue 60 | 0.4% | 84% | 88% | 88% |
| **C-13** | C.I. Disperse Yellow 23 | 1.1% | 86% | 86% | 86% |
| **C-14** | C.I. Solvent Yellow 163 | 1.5% | 90% | 90% | 90% |
| **C-15** | C.I. Disperse Blue 79 | 0.8% | 88% | 86% | 86% |
| **C-16** | C.I. Disperse Yellow 231 | 1.0% | 85% | 85% | 86% |
| **C-17** | C.I. Disperse Violet 63 | 0.5% | 85% | 85% | 86% |
| **C-18** | C.I. Disperse Blue 87 | 1.0% | 84% | 85% | 86% |
| **C-19** | C.I. Disperse Blue 291 | 1.0% | 88% | 86% | 86% |
| **C-20** | C.I. Disperse Blue 3 | 1.5% | 86% | 86% | 86% |
| **C-21** | C.I. Disperse Red 227 | 1.0% | 88% | 86% | 86% |
| **C-22** | C.I. Disperse Orange 13 | 0.8% | 85% | 85% | 86% |
| **C-23** | C.I. Disperse Red 72 | 1.5% | 90% | 90% | 90% |
| **C-24** | C.I. Disperse Orange 62 | 1.1% | 90% | 90% | 90% |
| **C-25** | C.I. Disperse Yellow 88 | 1.0% | 86% | 86% | 86% |
| **C-26** | C.I. Disperse Blue 85 | 2.5% | 85% | 88% | 88% |
| **C-27** | C.I. Disperse Blue 165 | 1.1% | 86% | 88% | 88% |
| **C-28** | C.I. Disperse Yellow 82 | 0.8% | 84% | 86% | 88% |
| **C-29** | C.I. Disperse Yellow 162 | 1.0% | 86% | 86% | 86% |
| **C-30** | C.I. Disperse Red 91 | 1.1% | 84% | 88% | 88% |
| **C-31** | C.I. Disperse Red 92 | 1.0% | 86% | 86% | 86% |
| **C-32** | C.I. Disperse Blue 94 | 1.5% | 86% | 88% | 89% |
| **C-33** | C.I. Disperse Yellow 93 | 1.0% | 85% | 85% | 86% |
| **C-34** | C.I. Disperse Orange 32 | 2.2% | 88% | 89% | 89% |

### EXAMPLE E-1 AND USE EXAMPLE E-A

1.5 parts of the dye C.I. Reactive Red 123 are dissolved in 100 parts of demineralized water and 8 parts of Glauber salt (calcined) are added. The dyebath is heated to 50°C and 10 parts of cotton fabric (bleached) are added. The temperature is maintained at 50°C during the addition of sodium carbonate. The dyebath is then heated to 60°C and the dyeing is continued at 60°C for one hour. The dyed fabric is then rinsed with running cold water for 3 minutes and then with running hot water for 3 minutes. The dyed fabric is then washed in boiling hot demineralized water in the presence of 0.25 part of Marseille soap for 15 minutes. After a further 3 minute rinse with running hot water and a subsequent centrifugation, the dyed fabric is dried in a drying cabinet at 70°C.

### USE EXAMPLE E-B

A dyebath containing 100 parts of demineralized water and 5 parts of Glauber salt is entered with 10 parts of cotton fabric (bleached).

The bath is then heated to 50°C over 10 minutes and subsequently 0.5 part of the abovementioned dye is added. After a further 30 minutes at 50°C 1 part of sodium carbonate (calcined) is added. The dyebath is then heated to 60°C and the dyeing is continued at 60°C for a further 45 minutes.

The dyed fabric is rinsed first with running cold water and then with hot water and subsequently washed as in Use Example E-A.

### USE EXAMPLE E-C

A printing paste consisting of

| | |
|---|---|
| 40 | parts of the abovementioned dye |
| 100 | parts of urea |
| 350 | parts of water |
| 500 | parts of a 4% sodium alginate thickener and |
| 10 | parts of sodium bicarbonate |
| 1000 | parts in total |

is applied to cotton fabric by known methods. The printed fabric is dried and fixed in steam at 102 - 104°C for 4 - 8 minutes.

It is then rinsed first with cold and then with hot water. It is subsequently washed in boiling water as described in Use Example E-A and then dried. The result is a violet dyeing having very good light and wet fastnesses, which is stable to oxidative influences.

### USE EXAMPLE E-D

2.5 parts of the abovementioned dye are stirred into a mixture of 20 parts of diethylene glycol and 77.5 parts of water at 25°C. The result is a printing ink useful for the inkjet printing process.

The reflectance of the dyed substrate compared with the undyed substrate in the near infrared region is:

| **Substrate** | **Dye** | **Concentration** | **Reflectance at 800 nm** | **950 nm** | **1100 nm** |
|---|---|---|---|---|---|
| Cotton interlock, bleached | --- | --- | 91% | 90% | 90% |
| Cotton interlock, bleached | C.I. Reactive Red 123 | 1.5% | 91% | 90% | 90% |

### EXAMPLES E-2 - E-23

Table 4 below contains dyes which were dyed or printed analogously to the Use Examples described under Example E1 using the appropriate dyeing auxiliaries, and also the reflectance values of the respective dyed or printed substrates in the near infrared region:

**TABLE 4**

| **Example** | **Substrate** | **Dye** | **Concentration** | **Reflectance at 800 nm** | **950 nm** | **1100 nm** |
|---|---|---|---|---|---|---|
| **E-2** | Cotton interlock, bleached | C.I. Reactive Black 5 | 2.0% | 91% | 90% | 90% |
| **E-3** | Cotton interlock, bleached | C.I. Reactive Black 39 | 2.0% | 91% | 92% | 92% |
| **E-4** | Cotton interlock, bleached | C.I. Reactive Yellow 13 | 3.0% | 91% | 92% | 92% |
| **E-5** | Cotton interlock, bleached | C.I. Reactive Yellow 174 | 1.8% | 92% | 93% | 92% |
| **E-6** | Cotton interlock, bleached | C.I. Reactive Red 198 | 2.0% | 91% | 92% | 92% |
| **E-7** | Cotton interlock, bleached | C.I. Reactive Red 241 | 2.2% | 91% | 92% | 92% |
| **E-8** | Cotton interlock, bleached | C.I. Reactive Blue 166 | 1.5% | 92% | 93% | 92% |
| **E-9** | Cotton interlock, bleached | C.I. Reactive Blue 225 | 2.0% | 91% | 92% | 92% |
| **E-10** | Cotton interlock, bleached | C.I. Reactive Blue 238 | 2.0% | 92% | 93% | 92% |
| **E-11** | Cotton interlock, bleached | C.I. Reactive Orange 12 | 1.8% | 90% | 92% | 92% |
| **E-12** | Cotton interlock, bleached | C.I. Reactive Orange 16 | 3.0% | 92% | 93% | 92% |
| **E-13** | Cotton interlock, bleached | C.I. Reactive Orange 64 | 2.8% | 91% | 92% | 92% |
| **E-14** | Cotton interlock, bleached | C.I. Reactive Orange 72 | 1.8% | 90% | 92% | 92% |
| **E-15** | Cotton interlock, bleached | C.I. Reactive Brown 2 | 2.0% | 92% | 93% | 92% |
| **E-16** | Cotton interlock, bleached | Drimaren Yellow HF-R | 2.0% | 92% | 93% | 92% |
| **E-17** | Cotton interlock, bleached | Drimaren Orange HF-2GL | 2.6% | 91% | 92% | 92% |
| **E-18** | Cotton interlock, bleached | Drimaren Scarlet HF-3G | 1.6% | 92% | 93% | 93% |
| **E-19** | Cotton interlock, bleached | Drimaren Red HF-G | 1.9% | 91% | 92% | 92% |
| **E-20** | Cotton interlock, bleached | Drimaren Red HF-2B | 3.7% | 91% | 92% | 92% |
| **E-21** | Cotton interlock, bleached | Drimaren Brown HF-2RL | 3.2% | 91% | 92% | 92% |
| **E-22** | Cotton interlock, bleached | Drimaren Navy HF-B | 1.0% | 89% | 91% | 91% |
| **E-23** | Cotton interlock, bleached | Drimaren Navy HF-G | 1.8% | 89% | 91% | 91% |

## Claims

1. Use of dyes for the type of fibre in question for minimally reducing, retaining or increasing the NIR reflectance, in the region of electromagnetic radiation of wavelength 700 nm to 1100 nm of textile material in relation to the undyed and untreated textile material, **characterized in that** customary dyeing and/or printing processes for the type of fibre in question are used and **characterized in that** the dyes are metal-free and have one of the following structures (A-I), (A-II), (A-III), (A-IV) or (A-V) where
A is an unsubstituted or substituted naphthyl radical or an unsubstituted or substituted phenyl radical,
R³² is hydrogen, hydroxyl, amino or an unsubstituted or substituted naphthyl radical or an unsubstituted or substituted phenyl radical, and
n is 1, 2 or 3.
where
A is an unsubstituted or substituted naphthyl radical or an unsubstituted or substituted phenyl radical,
R³³ is hydrogen, hydroxyle, amino or an unsubstituted or substituted naphthyl radical or an unsubstituted or substituted phenyl radical, and
n is 1, 2 or 3.
where
R³⁴, R³⁵, R³⁶, R³⁷ are each hydrogen, hydroxyl, amino, substituted or unsubstituted C₁ to C₄ alkyl, or an unsubstituted or substituted naphthyl radical or an unsubstituted or substituted phenyl radical and the dye of formula A-(III) bears one, two or three sulpho groups.
where
A, R³⁸, R³⁹ are each hydrogen, hydroxyl, amino, substituted or unsubstituted C₁ to C₄ alkyl, or an unsubstituted or substituted naphthyl radical or an unsubstituted or substituted phenyl radical and the dye of formula A-(IV) bears one, two or three sulpho groups.
where
R⁴⁰, R⁴¹, R⁴² are each hydrogen, hydroxyl, amino, substituted or unsubstituted C₁ to C₄ alkyl, or an unsubstituted or substituted naphthyl radical or an unsubstituted or substituted phenyl radical,
m is 0, 1, 2 or 3 and the dye of formula (A-V) bears one, two or three sulpho groups.
or have one of the following structures (B-I), (B-II), (B-III), (B-IV) where
R⁴³ and R⁴⁴ are independently substituted or unsubstituted C₁ to C₄ alkyl, substituted or unsubstituted -(C₁₋₄ alkylene)-N⁺-(C₁₋₄alkyl)₂, the dye of the formula (B-I) being at least singly or doubly positively charged;
where
R⁵⁵ and R⁵⁶ are independently substituted or unsubstituted C₁ to C₄ alkyl, substituted or unsubstituted -N-(C₁₋₄ alkyl)₂;
where
R⁵⁷ and R⁵⁸ are independently substituted or unsubstituted phenyl, substituted or unsubstituted naphthyl, and
R⁵⁹ is independently substituted or unsubstituted phenyl, substituted or unsubstituted naphthyl or =N⁺H₂;
where
R⁶⁰ is (C₁₋₄ alkyl)-C(O)NH₂
R⁶¹ is C₁₋₄ alkyl or C₁₋₄ alkoxy, and
R⁶² is substituted or un substituted phenyl, substituted or unsubstituted naphthyl.
or have the following dyes of the formula (C-1) or (C-2) or (C-3) or (C-4) or (C-5) or (C-6) or (C-7) or (C-8) or (C-9) or (C-10) or (C-11) or (C-12): where
R₁ is hydrogen, halogen, nitro or cyano
R₂ is hydrogen, halogen, nitro or cyano
R₃ is hydrogen, halogen, C₁-C₄-alkoxy or C₁-C₄-alkyl
R₄ is hydrogen, C₁-C₄-alkyl,
R₅ is hydrogen, unsubstituted or hydroxyl-, cyano-, C₁-C₄-alkylcarbonyloxy-substituted C₁-C₄-alkyl or C₁-C₄-alkenyl,
R₆ is unsubstituted or hydroxyl-, cyano-, C₁-C₄-alkylcarbonyloxy-, C₁-C₄-alkoxycarbonyl-substituted C₁-C₄-alkyl or C₁-C₄-alkenyl,
R₇ is nitro, C₁-C₄-alkoxy or the radical -SO₂CH₃,
R₈ is hydrogen or C₁-C₄-alkyl,
R₉ is hydrogen or C₁-C₄-alkyl,
R₁₀ is unsubstituted or hydroxyl- or cyano-substituted C₁-C₄-alkyl,
R₁₁ is unsubstituted C₁-C₄-alkyl or C₁-C₄-alkyl substituted by the radical -O-COR₁₂, where R₁₂ is C₁-C₄-alkyl;
where
R₁₃ is C₁-C₄-alkyl,
R₁₄ is C₁-C₄-alkyl, and
Halogen represents the halogen atoms; where the rings A and B may be further substituted; where
R₁₅ is C₁-C₄-alkyl and
the rings C and D may be further substituted; where
R₁₆ is unsubstituted or hydroxyl- or cyano-substituted C₁-C₄-alkyl,
R₁₇ is unsubstituted C₁-C₄-alkyl or C₁-C₄-alkyl substituted by the radical -O-COR₁₈, where R₁₈ is C₁-C₄-alkyl,
R₃₂ is nitro, C₁-C₄-alkoxy or the radical -SO₂CH₃, and
R₃₃ is hydrogen or C₁-C₄-alkyl;
where
R₁₉ is C₁-C₄-alkyl,
R₂₀ is C₁-C₄-alkyl,
R₂₁ is C₁-C₄-alkyl, and
R₂₂ is C₁-C₄-alkyl or the radical -NHCOR₂₃ where R₂₃ is C₁-C₄-alkyl;
where R₂₄ is halogen; where
R₂₅ is cyano, nitro or halogen,
R₂₆ is halogen,
R₂₇ is unsubstituted or hydroxyl-substituted C₁-C₄-alkyl, and
R₂₈ is unsubstituted or hydroxyl-substituted C₁-C₄-alkyl, and
the naphthyl ring E may be further substituted, and/or where
R₂₉ is C₁-C₄-alkyl or the radical NHCOR₁₇ where R₁₇ is C₁-C₄-alkyl,
R₃₀ is C₁-C₄-alkyl or C₁-C₄-alkylcarbonyloxy-C₁-C₄-alkyl, and
R₃₁ is C₁-C₄-alkyl or C₁-C₄-alkylcarbonyloxy-C₁-C₄-alkyl
or have one of the following structures (E-I), (E-II), (E-III), (E-IV), (E-V) or (E-VI) where
A is an unsubstituted or substituted naphthyl radical or an unsubstituted or substituted phenyl radical,
R⁶³ is hydrogen, hydroxyl, amino, an amine substituted by unsubstituted or substituted naphthyl or by unsubstituted or substituted phenyl, or an unsubstituted or substituted naphthyl radical or an unsubstituted or substituted phenyl radical,
n is 1 or 2 and the dye of formula (E-I) bears one or two fibre-reactive groups;
where
A is an unsubstituted or substituted naphthyl radical or an unsubstituted or substituted phenyl radical,
R⁶⁴ is hydrogen, hydroxyl, amino, an amine substituted by unsubstituted or substituted naphthyl or by unsubstituted or substituted phenyl, or an unsubstituted or substituted naphthyl radical or an unsubstituted or substituted phenyl radical,
n is 1, 2 or 3 and the dye of formula (E-II) bears one or two fibre-reactive groups;
where
R⁶⁵, R⁶⁶, R⁶⁷, R⁶⁸ are each hydrogen, hydroxyl, amino, substituted or unsubstituted C₁ to C₄ alkyl, or an unsubstituted or substituted naphthyl radical or an unsubstituted or substituted phenyl radical and the dye of formula (E-III) bears one, two or three sulpho groups and also one or two fibre-reactive groups;
where
A, R⁶⁹, R⁷⁰ are each hydrogen, hydroxyl, amino, an amine substituted by unsubstituted or substituted naphthyl or by unsubstituted or substituted phenyl, or an unsubstituted or substituted naphthyl radical or an unsubstituted or substituted phenyl radical and the dye of formula (E-IV) bears one, two or three sulpho groups and also one or two fibre-reactive groups;
where
R⁷¹, R⁷² R⁷³ are each hydrogen, hydroxyl, amino, substituted or unsubstituted C₁ to C₄ alkyl, or an unsubstituted or substituted naphthyl radical or an unsubstituted or substituted phenyl radical
m is 0, 1, 2 or 3 and the dye of formula (E-V) bears one, two or three sulpho groups and also one or two fibre-reactive groups;
where
A in each occurrence is independently an unsubstituted or substituted naphthyl radical or an unsubstituted or substituted phenyl radical,
R⁷⁴ is hydroxyl, amino, an amine substituted by unsubstituted or substituted naphthyl or by unsubstituted or substituted phenyl, or an unsubstituted or substituted naphthyl radical or an unsubstituted or substituted phenyl radical,
n is 1 or 2 and the dye of formula (E-VI) bears one or two fibre-reactive groups

2. Use according to Claim 1, **characterized in that** the NIR reflectance, in the region of electromagnetic radiation of wavelength 700 nm to 1100 nm of textile material in relation to the undyed and untreated textile material is increased.

## Patentansprüche

1. Verwendung von Farbstoffen für die betreffende Faserart zur geringen Erniedrigung, Beibehaltung oder Erhöhung der NIR-Remission im Bereich von elektromagnetischer Strahlung mit Wellenlänge von 700 nm bis 1100 nm von Textilmaterial in Bezug auf das ungefärbte und unbehandelte Textilmaterial, **dadurch gekennzeichnet, dass** für die betreffende Faserart übliche Färbe- und/oder Druckverfahren verwendet werden, und **dadurch gekennzeichnet, dass** die Farbstoffe metallfrei sind und eine der folgenden Strukturen (A-I), (A-II), (A-III), (A-IV) oder (A-V) haben: wobei
A für einen unsubstituierten oder substituierten Naphthylrest oder einen unsubstituierten oder substituierten Phenylrest steht,
R³² für Wasserstoff, Hydroxy, Amino oder einen unsubstituierten oder substituierten Naphthylrest oder einen unsubstituierten oder substituierten Phenylrest steht und
n für 1, 2 oder 3 steht.
wobei
A für einen unsubstituierten oder substituierten Naphthylrest oder einen unsubstituierten oder substituierten Phenylrest steht,
R³³ für Wasserstoff, Hydroxy, Amino oder einen unsubstituierten oder substituierten Naphthylrest oder einen unsubstituierten oder substituierten Phenylrest steht und
n für 1, 2 oder 3 steht.
wobei
R³⁴ , R³⁵ , R³⁶ , R³⁷ jeweils für Wasserstoff, Hydroxy, Amino, substituiertes oder unsubstituiertes C₁- bis C₄-Alkyl oder einen unsubstituierten oder substituierten Naphthylrest oder einen unsubstituierten oder substituierten Phenylrest stehen und der Farbstoff der Formel (A-III) eine, zwei oder drei Sulfogruppen trägt.
wobei
A, R³⁸, R³⁹ jeweils für Wasserstoff, Hydroxy, Amino, substituiertes oder unsubstituiertes C₁- bis C₄-Alkyl oder einen unsubstituierten oder substituierten Naphthylrest oder einen unsubstituierten oder substituierten Phenylrest stehen und der Farbstoff der Formel (A-IV) eine, zwei oder drei Sulfogruppen trägt.
wobei
R⁴⁰, R⁴¹, R⁴² jeweils für Wasserstoff, Hydroxy, Amino, substituiertes oder unsubstituiertes C₁- bis C₄-Alkyl oder einen unsubstituierten oder substituierten Naphthylrest oder einen unsubstituierten oder substituierten Phenylrest stehen,
m für 0, 1, 2 oder 3 steht und der Farbstoff der Formel (A-V) eine, zwei oder drei Sulfogruppen trägt.
oder eine der folgenden Strukturen (B-I), (B-II), (B-III), (B-IV) haben: wobei
R⁴³ und R⁴⁴ unabhängig voneinander für substituiertes oder unsubstituiertes C₁- bis C₄-Alkyl, substituiertes oder unsubstituiertes -(C₁₋₄-Alkylen)-N⁺-(C₁₋₄-alkyl)₂ stehen, wobei der Farbstoff der Formel (B-I) mindestens einfach oder zweifach positiv geladen ist;
wobei
R⁵⁵ und R⁵⁶ unabhängig voneinander für substituiertes oder unsubstituiertes C₁- bis C₄-Alkyl, substituiertes oder unsubstituiertes -N-(C₁-₄-Alkyl)₂ stehen,
wobei
R⁵⁷ und R⁵⁸ unabhängig voneinander für substituiertes oder unsubstituiertes Phenyl, substituiertes oder unsubstituiertes Naphthyl stehen und
R⁵⁹ unabhängig voneinander für substituiertes oder unsubstituiertes Phenyl, substituiertes oder unsubstituiertes Naphthyl oder =N⁺H₂ steht;
wobei
R⁶¹ für (C₁₋₄-Alkyl)-C(O)NH₂ steht,
R⁶¹ für C₁₋₄-Alkyl oder C₁₋₄-Alkoxy steht und
R⁶² für substituiertes oder unsubstituiertes Phenyl, substituiertes oder unsubstituiertes Naphthyl steht.
oder die folgenden Farbstoffe der Formel (C-1) oder (C-2) oder (C-3) oder (C-4) oder (C-5) oder (C-6) oder (C-7) oder (C-8) oder (C-9) oder (C-10) oder (C-11) oder (C-12) haben: wobei
R₁ für Wasserstoff, Halogen, Nitro oder Cyano steht,
R₂ für Wasserstoff, Halogen, Nitro oder Cyano steht,
R₃ für Wasserstoff, Halogen, C₁-C₄-Alkoxy oder C₁-C₄-Alkyl steht,
R₄ für Wasserstoff, C₁-C₄-Alkyl steht,
R₅ für Wasserstoff, unsubstituiertes oder durch Hydroxy, Cyano, C₁-C₄-Alkylcarbonyloxy substituiertes C₁-C₄-Alkyl oder C₁-C₄-Alkenyl steht,
R₆ für unsubstituiertes oder durch Hydroxy, Cyano, C₁-C₄-Alkylcarbonyloxy, C₁-C₄-Alkoxycarbonyl substituiertes C₁-C₄-Alkyl oder C₁-C₄-Alkenyl steht,
R₇ für Nitro, C₁-C₄-Alkoxy oder den Rest -SO₂CH₃ steht,
R₈ für Wasserstoff oder C₁-C₄-Alkyl steht,
R₉ für Wasserstoff oder C₁-C₄-Alkyl steht,
R₁₀ für unsubstituiertes oder durch Hydroxy oder Cyano substituiertes C₁-C₄-Alkyl steht,
R₁₁ für unsubstituiertes oder durch den Rest -O-COR₁₂ substituiertes C₁-C₄-Alkyl mit R₁₂ in der Bedeutung C₁-C₄-Alkyl steht;
wobei
R₁₃ für C₁-C₄-Alkyl steht,
R₁₄ für C₁-C₄-Alkyl steht und
Halogen für die Halogenatome steht; wobei die Ringe A und B weiter substituiert sein können; wobei
R₁₅ für C₁-C₄-Alkyl steht und
die Ringe C und D weiter substituiert sein können; wobei
R₁₆ für unsubstituiertes oder durch Hydroxy oder Cyano substituiertes C₁-C₄-Alkyl steht,
R₁₇ für unsubstituiertes oder durch den Rest -O-COR₁₈ substituiertes C₁-C₄-Alkyl mit R₁₈ in der Bedeutung C₁-C₄-Alkyl steht,
R₃₂ für Nitro, C₁-C₄-Alkoxy oder den Rest -SO₂CH₃ steht und
R₃₃ für Wasserstoff oder C₁-C₄-Alkyl steht;
wobei
R₁₉ für C₁-C₄-Alkyl steht,
R₂₀ für C₁-C₄-Alkyl steht,
R₂₁ für C₁-C₄-Alkyl steht und
R₂₂ für C₁-C₄-Alkyl oder den Rest -NHCOR₂₃ mit R₂₃ in der Bedeutung C₁-C₄-Alkyl steht;
wobei R₂₄ für Halogen steht; wobei
R₂₅ für Cyano, Nitro oder Halogen steht,
R₂₆ für Halogen steht,
R₂₇ für unsubstituiertes oder durch Hydroxy substituiertes C₁-C₄-Alkyl steht und
R₂₈ für unsubstituiertes oder durch Hydroxy substituiertes C₁-C₄-Alkyl steht und
der Naphthylring E weiter substituiert sein kann, und/oder wobei
R₂₉ für C₁-C₄-Alkyl oder den Rest NHCOR₁₇ mit R₁₇ in der Bedeutung C₁-C₄-Alkyl steht,
R₃₀ für C₁-C₄-Alkyl oder C₁-C₄-Alkylcarbonyloxy-C₁-C₄-alkyl steht und
R₃₁ für C₁-C₄-Alkyl oder C₁-C₄-Alkylcarbonyloxy-C₁-C₄-alkyl steht;
oder eine der folgenden Strukturen (E-I), (E-II), (E-III), (E-IV), (E-V) oder (E-VI) haben: wobei
A für einen unsubstituierten oder substituierten Naphthylrest oder einen unsubstituierten oder substituierten Phenylrest steht,
R⁶³ für Wasserstoff, Hydroxy, Amino, ein durch einen unsubstituierten oder substituierten Naphthylrest oder einen unsubstituierten oder substituierten Phenylrest substituiertes Amin oder einen unsubstituierten oder substituierten Naphthylrest oder einen unsubstituierten oder substituierten Phenylrest steht,
n für 1 oder 2 steht und der Farbstoff der Formel (E-I) eine oder zwei faserreaktive Gruppen trägt;
wobei
A für einen unsubstituierten oder substituierten Naphthylrest oder einen unsubstituierten oder substituierten Phenylrest steht,
R⁶⁴ für Wasserstoff, Hydroxy, Amino, ein durch einen unsubstituierten oder substituierten Naphthylrest oder einen unsubstituierten oder substituierten Phenylrest substituiertes Amin oder einen unsubstituierten oder substituierten Naphthylrest oder einen unsubstituierten oder substituierten Phenylrest steht,
n für 1, 2 oder 3 steht und der Farbstoff der Formel (E-II) eine oder zwei faserreaktive Gruppen trägt;
wobei
R⁶⁵, R⁶⁶, R⁶⁷, R⁶⁸ jeweils für Wasserstoff, Hydroxy, Amino, substituiertes oder unsubstituiertes C₁- bis C₄-Alkyl oder einen unsubstituierten oder substituierten Naphthylrest oder einen unsubstituierten oder substituierten Phenylrest stehen und der Farbstoff der Formel (E-III) eine, zwei oder drei Sulfogruppen sowie eine oder zwei faserreaktive Gruppen trägt;
wobei
A, R⁶⁹, R⁷⁰ jeweils für Wasserstoff, Hydroxy, Amino, ein durch einen unsubstituierten oder substituierten Naphthylrest oder einen unsubstituierten oder substituierten Phenylrest substituiertes Amin oder einen unsubstituierten oder substituierten Naphthylrest oder einen unsubstituierten oder substituierten Phenylrest stehen und der Farbstoff der Formel (E-IV) eine, zwei oder drei Sulfogruppen sowie eine oder zwei faserreaktive Gruppen trägt;
wobei
R⁷¹, R⁷² , R⁷³ jeweils für Wasserstoff, Hydroxy, Amino, substituiertes oder unsubstituiertes C₁- bis C₄-Alkyl oder einen unsubstituierten oder substituierten Naphthylrest oder einen unsubstituierten oder substituierten Phenylrest stehen,
m für 0, 1, 2 oder 3 steht und der Farbstoff der Formel (E-V) eine, zwei oder drei Sulfogruppen sowie eine oder zwei faserreaktive Gruppen trägt;
wobei
A jeweils unabhängig voneinander für einen unsubstituierten oder substituierten Naphthylrest oder einen unsubstituierten oder substituierten Phenylrest steht,
R⁷⁴ für Hydroxy, Amino, ein durch einen unsubstituierten oder substituierten Naphthylrest oder einen unsubstituierten oder substituierten Phenylrest substituiertes Amin oder einen unsubstituierten oder substituierten Naphthylrest oder einen unsubstituierten oder substituierten Phenylrest steht,
n für 1 oder 2 steht und der Farbstoff der Formel (E-VI) eine oder zwei faserreaktive Gruppen trägt.

2. Verwendung nach Anspruch 1, **dadurch gekennzeichnet, dass** die NIR-Remission im Bereich von elektromagnetischer Strahlung mit Wellenlänge von 700 nm bis 1100 nm von Textilmaterial in Bezug auf das ungefärbte und unbehandelte Textilmaterial erhöht wird.

## Revendications

1. Utilisation de colorants pour le type de fibre en question pour la réduction au minimum, le maintien ou l'augmentation du facteur de réflexion dans le proche infrarouge, dans le domaine du rayonnement électromagnétique ayant une longueur d'onde de 700 nm à 1100 nm, d'une matière textile par rapport à la matière textile non teinte et non traitée, **caractérisée en ce que** des procédés de teinture et/ou d'impression usuels pour le type de fibre en question sont utilisés et **caractérisée en ce que** les colorants sont exempts de métaux et ont l'une des structures (A-I), (A-II), (A-III), (A-IV) ou (A-V) suivantes où
A est un radical naphtyle non substitué ou substitué ou un radical phényle non substitué ou substitué,
R³² est l'atome d'hydrogène, le groupe hydroxyle, le groupe amino ou un radical naphtyle non substitué ou substitué ou un radical phényle non substitué ou substitué et
n vaut 1, 2 ou 3 ;
où
A est un radical naphtyle non substitué ou substitué ou un radical phényle non substitué ou substitué,
R³³ est l'atome d'hydrogène, le groupe hydroxyle, le groupe amino ou un radical naphtyle non substitué ou substitué ou un radical phényle non substitué ou substitué et
n vaut 1, 2 ou 3 ;
où
R³⁴, R³⁵ , R³⁶ et R³⁷ sont chacun l'atome d'hydrogène, le groupe hydroxyle, le groupe amino, un groupe alkyle en C₁ à C₄ substitué ou non substitué ou un radical naphtyle non substitué ou substitué ou un radical phényle non substitué ou substitué et
le colorant de formule (A-III) porte un, deux ou trois groupes sulfo ; où
A, R³⁸ et R³⁹ sont chacun l'atome d'hydrogène, le groupe hydroxyle, le groupe amino, un groupe alkyle en C₁ à C₄ substitué ou non substitué ou un radical naphtyle non substitué ou substitué ou un radical phényle non substitué ou substitué et
le colorant de formule (A-IV) porte un, deux ou trois groupes sulfo ; où
R⁴⁰, R⁴¹ et R⁴² sont chacun l'atome d'hydrogène, le groupe hydroxyle, le groupe amino, un groupe alkyle en C₁ à C₄ substitué ou non substitué ou un radical naphtyle non substitué ou substitué ou un radical phényle non substitué ou substitué,
m vaut 0, 1, 2 ou 3 et
le colorant de formule (A-V) porte un, deux ou trois groupes sulfo ;
ou ont l'une des structures (B-I), (B-II), (B-III) ou (B-IV) suivantes où
R⁴³ et R⁴⁴ sont chacun indépendamment un groupe alkyle en C₁ à C₄ substitué ou non substitué ou un groupe -(alkylène en C₁₋₄)-N⁺-(alkyle en C₁₋₄)₂ substitué ou non substitué,
le colorant représenté par la formule (B-I) portant au moins une charge unique ou double ; où
R⁵⁵ et R⁵⁶ sont chacun indépendamment un groupe alkyle en C₁ à C₄ substitué ou non substitué ou un groupe -N-(alkyle en C₁₋₄)₂ substitué ou non substitué ;
où
R⁵⁷ et R⁵⁸ sont chacun indépendamment un groupe phényle substitué ou non substitué ou un groupe naphtyle substitué ou non substitué et
R⁵⁹ est indépendamment un groupe phényle substitué ou non substitué, un groupe naphtyle substitué ou non substitué ou =N⁺H₂ ;
où
R⁶⁰ est un groupe (alkyl en C₁-₄)-C(O)NH₂.
R⁶¹ est un groupe alkyle en C₁₋₄ ou un groupe alcoxy en C₁₋₄ et
R⁶² est un groupe phényle substitué ou non substitué ou un groupe naphtyle substitué ou non substitué ;
ou ont les colorants suivants représentés par la formule (C-1) ou (C-2) ou (C-3) ou (C-4) ou (C-5) ou (C-6) ou (C-7) ou (C-8) ou (C-9) ou (C-10) ou (C-11) ou (C-1 2) : où
R₁ est l'atome d'hydrogène, un atome d'halogène, le groupe nitro ou le groupe cyano,
R₂ est l'atome d'hydrogène, un atome d'halogène, le groupe nitro ou le groupe cyano,
R₃ est l'atome d'hydrogène, un atome d'halogène, un groupe alcoxy en C₁-C₄ ou un groupe alkyle en C₁-C₄,
R₄ est l'atome d'hydrogène ou un groupe alkyle en C₁-C₄,
R₅ est l'atome d'hydrogène, un groupe alkyle en C₁-C₄ non substitué ou substitué par hydroxyle, cyano ou (alkyl en C₁-C₄)carbonyloxy ou un groupe alcényle en C₁-C₄,
R₆ est un groupe alkyle en C₁-C₄ non substitué ou substitué par hydroxyle, cyano, (alkyl en C₁-C₄)carbonyloxy ou (alcoxy en C₁-C₄)carbonyle ou un groupe alcényle en C₁-C₄,
R₇ est le groupe nitro, un groupe alcoxy en C₁-C₄ ou le radical - SO₂CH₃,
R₈ est l'atome d'hydrogène ou un groupe alkyle en C₁-C₄,
R₉ est l'atome d'hydrogène ou un groupe alkyle en C₁-C₄,
R₁₀ est un groupe alkyle en C₁-C₄ non substitué ou substitué par hydroxyle ou cyano,
R₁₁ est un groupe alkyle en C₁-C₄ non substitué ou un groupe alkyle en C₁-C₄ substitué par le radical -O-COR₁₂, où R₁₂ est un groupe alkyle en C₁-C₄ ;
où
R₁₃ est un groupe alkyle en C₁-C₄,
R₁₄ est un groupe alkyle en C₁-C₄ et
halogène représente les atomes d'halogène ; où
les noyaux A et B peuvent être encore substitués ; où
R₁₅ est un groupe alkyle en C₁-C₄ et
les noyaux C et D peuvent être encore substitués ; où
R₁₆ est un groupe alkyle en C₁-C₄ non substitué ou substitué par hydroxyle ou cyano,
R₁₇ est un groupe alkyle en C₁-C₄ non substitué ou un groupe alkyle en C₁-C₄ substitué par le radical -O-COR₁₈, où R₁₈ est un groupe alkyle en C₁-C₄,
R₃₂ est le groupe nitro, un groupe alcoxy en C₁-C₄ ou le radical - SO₂CH₃ et
R₃₃ est l'atome d'hydrogène ou un groupe alkyle en C₁-C₄ ;
où
R₁₉ est un groupe alkyle en C₁-C₄,
R₂₀ est un groupe alkyle en C₁-C₄.
R₂₁ est un groupe alkyle en C₁-C₄ et
R₂₂ est un groupe alkyle en C₁-C₄ ou le radical -NHCOR₂₃ où R₂₃ est un groupe alkyle en C₁-C₄ ;
où
R₂₄ est un atome d'halogène ;
où
R₂₅ est le groupe cyano, le groupe nitro ou un atome d'halogène,
R₂₆ est un atome d'halogène,
R₂₇ est un groupe alkyle en C₁-C₄ non substitué ou substitué par hydroxyle et
R₂₈ est un groupe alkyle en C₁-C₄ non substitué ou substitué par hydroxyle et
le noyau naphtyle E peut être encore substitué ;
et/ou où
R₂₉ est un groupe alkyle en C₁-C₄ ou le radical -NHCOR₁₇ où R₁₇ est un groupe alkyle en C₁-C₄,
R₃₀ est un groupe alkyle en C₁-C₄ ou (alkyl en C₁-C₄)carbonyloxy-(alkyle en C₁-C₄) et
R₃₁ est un groupe alkyle en C₁-C₄ ou (alkyl en C₁-C₄)carbonyloxy-(alkyle en C₁-C₄);
ou ont l'une des structures (E-I), (E-II), (E-III), (E-IV), (E-V) ou (E-VI) suivantes où
A est un radical naphtyle non substitué ou substitué ou un radical phényle non substitué ou substitué,
R⁶³ est l'atome d'hydrogène, le groupe hydroxyle, le groupe amino, une amine substituée par naphtyle non substitué ou substitué ou par phényle non substitué ou substitué ou un radical naphtyle non substitué ou substitué ou un radical phényle non substitué ou substitué,
n vaut 1 ou 2 et
le colorant de formule (E-I) porte un ou deux groupes réactifs avec les fibres ; où
A est un radical naphtyle non substitué ou substitué ou un radical phényle non substitué ou substitué,
R⁶⁴ est l'atome d'hydrogène, le groupe hydroxyle, le groupe amino, une amine substituée par naphtyle non substitué ou substitué ou par phényle non substitué ou substitué ou un radical naphtyle non substitué ou substitué ou un radical phényle non substitué ou substitué,
n vaut 1, 2 ou 3 et
le colorant de formule (E-II) porte un ou deux groupes réactifs avec les fibres ; où
R⁶⁵ , R⁶⁶ , R⁶⁷ et R⁶⁸ sont chacun l'atome d'hydrogène, le groupe hydroxyle, le groupe amino, un groupe alkyle en C₁ à C₄ substitué ou non substitué ou un radical naphtyle non substitué ou substitué ou un radical phényle non substitué ou substitué et
le colorant de formule (E-III) porte un, deux ou trois groupes sulfo et également un ou deux groupes réactifs avec les fibres ; où
A, R⁶⁹ et R⁷⁰ sont chacun l'atome d'hydrogène, le groupe hydroxyle, le groupe amino, une amine substituée par naphtyle non substitué ou substitué ou par phényle non substitué ou substitué ou un radical naphtyle non substitué ou substitué ou un radical phényle non substitué ou substitué et
le colorant de formule (E-IV) porte un, deux ou trois groupes sulfo et également un ou deux groupes réactifs avec les fibres ; où
R⁷¹ , R⁷² et R⁷³ sont chacun l'atome d'hydrogène, le groupe hydroxyle, le groupe amino, un groupe alkyle en C₁ à C₄ substitué ou non substitué ou un radical naphtyle non substitué ou substitué ou un radical phényle non substitué ou substitué,
m vaut 0, 1, 2 ou 3 et
le colorant de formule (E-V) porte un, deux ou trois groupes sulfo et également un ou deux groupes réactifs avec les fibres ; où
A est à chaque fois indépendamment un radical naphtyle non substitué ou substitué ou un radical phényle non substitué ou substitué,
R⁷⁴ est le groupe hydroxyle, le groupe amino, une amine substituée par naphtyle non substitué ou substitué ou par phényle non substitué ou substitué ou un radical naphtyle non substitué ou substitué ou un radical phényle non substitué ou substitué,
n vaut 1 ou 2 et
le colorant de formule (E-VI) porte un ou deux groupes réactifs avec les fibres.

2. Utilisation selon la revendication 1, **caractérisée en ce que** le facteur de réflexion dans le proche infrarouge, dans le domaine du rayonnement électromagnétique ayant une longueur d'onde de 700 nm à 1100 nm, de la matière textile par rapport à la matière textile non teinte et non traitée est accru.
